

## UNITED STATES PATENT OFFICE

2,638,665

## METHOD OF WELDING STAINLESS STEEL

Prentiss S. Viles, Baytown, Tex., assignor, by  
mesne assignments, to Standard Oil Develop-  
ment Company, Elizabeth, N. J., a corporation  
of Delaware

No Drawing. Application October 23, 1950,  
Serial No. 191,725

6 Claims. (Cl. 29—351)

1

The present invention is directed towards a method for welding ferrous alloys comprising substantially chromium, iron and nickel and referred to in the trade as stainless steels. More specifically the invention is directed toward the prevention of corrosion due to welding of stainless steels which frequently manifests itself as an after effect when the welded stainless steels are employed.

This application is a continuation-in-part of Serial No. 716,669, now abandoned, filed December 16, 1946, for Prentiss S. Viles and entitled "Method for Welding Stainless Steel."

The chromium nickel stainless steels are those containing nickel and chromium plus other elements to a lesser degree. These chromium nickel stainless steels are known as the austenitic chromium-nickel stainless steels, the nickel being added in sufficient amount to make the steels austenitic and nonmagnetic with improved ductility and conductiveness over the straight chromium steels.

These austenitic steels are outstanding in their resistance to corrosion and oxidation. Because of their excellent physical properties both at low and elevated temperatures they find wide application in the food, pulp, paper, textile, dye, chemical, oil refining and other related industries. The severe corrosion encountered in the use of these alloys, however, introduces many perplexing problems and many uses will demand a selection among the various types of steel available.

The corrosion characteristics of the steel are affected not only by the media in contact with the structural material but by the treatment the steel is given in its fabrication into structural shapes and facilities. In fabricating containers, pipes and various structural shapes and equipment it is necessary to employ welding. During the welding operation the stainless steel may be subjected to temperatures between 800° and 1600° F. whether the welding be accomplished by the oxy-acetylene, atomic hydrogen, or by the electric arc methods. When the austenitic chromium nickel steels are subjected to temperatures between 800° and 1600° F. as occurs during welding, a structural change is effected in the steels. The carbon migrates out from the solid solution and combines with the chromium to form chromium carbides along the grain boundaries. This effect is known as carbide precipitation and this action impoverishes the chromium content adjacent to the grain boundaries; this increases the susceptibility to corrosion attack and leads to

2

what is generally referred to as intergranular corrosion at the grain boundaries.

The precipitation of carbide is affected by a number of factors among which is the time the material is held within the critical temperature range. The longer the heat treatment the more carbides precipitate and as the temperature approaches 1200° F. the more undesirable will be the structural change in the steel. It follows that the higher carbon content steels are more susceptible to carburization since there is more carbon available to combine with the chromium.

The problem of carbide precipitation and corrosion by intergranular attack has been solved in the industry by subjecting the welded metal to a heat treatment. The heat treatment involves heating the metal to a temperature between 1900° and 2000° F. for a sufficient time to allow the chromium carbides to redissolve and go back into solution. Following the heat treatment the steel is quickly cooled by quenching with water or by air blasts or other suitable means. It is necessary to cool the heat treated material rapidly through the temperature range between 1600° and 800° F. to avoid the possibility of carbides forming again in passing through the critical temperature region.

Another method of suppressing the formation of chromium carbides in welding involves addition of several of the rare metals such as columbium and the like to the metals to act as stabilizers. These materials combine with the carbon and prevent or retard the formation of objectionable chromium carbides and thus reduce the tendency to intergranular corrosion.

The prior art methods in overcoming the formation of chromium carbides in the welding of stainless steels is expensive in that furnaces for the heat treatment must be provided which may also contribute to the cost of the steel. Too, even with the addition of stabilizer metals, carbide formation may be encountered.

It is, therefore, the main object of the present invention to provide a method of welding austenitic stainless steel alloys which will substantially reduce or prevent the precipitation of chromium carbides at the grain boundaries of the metal and thus reduce the susceptibility of the welded material to intergranular corrosion.

In accordance with the present invention the precipitation of carbides during welding operations with its attendant degradation in the quality of the steel is materially reduced or substantially eliminated by the employment of a retarding agent during the welding operation. The

carburization retarding agent employed in the present invention is elementary sulfur which is incorporated into the welding flux and which may be applied to adjacent boundaries of metals which are being welded or may be employed as a coating on the welding rod which is customarily used in weld operations. It is contemplated that the amount of elementary sulfur employed in the practice of the present invention may range from 0.25% to 25% by weight of the welding flux. Lesser quantities give welds which show evidence of carbide precipitation while larger amounts may be impractical.

In order to illustrate the effectiveness of the present invention, a number of welds were made employing 18-8 steel alloys. Adjacent boundaries of the bodies of the alloys were welded together in accordance with conventional welding techniques. In the first weld a conventional flux was employed. In the following welds a conventional flux was employed except that amounts ranging from 0.1% to 25% by weight of elementary sulfur was incorporated in the flux and applied to the region of the adjacent boundaries of metals being welded. These welded strips were then tested for intergranular corrosion by the Straus test. The Straus test consists of immersing the specimens in boiling Straus solution (3% cupric sulfate, 10% sulfuric acid and 87% distilled water) for 72 hours and then bending the specimen 180°. The Straus test is a method for determining the extent of carbide precipitation in metals and a description thereof may be found in the Welding Handbook, 1938 edition, American Welding Society, N. Y. pages 533-4.

The following table shows the condition of the several welds after testing for metal loss in the Straus test.

Table

| Metal Welded                | Weight Percent Sulfur in Flux | Straus Test—72 Hours |                            |
|-----------------------------|-------------------------------|----------------------|----------------------------|
|                             |                               | Metal Loss, Percent  | Condition After 180° Bend  |
| 18-8, Type 304 <sup>1</sup> | 0                             | 1.97                 | Broken, granular cracks.   |
| Do                          | 0.1                           | 0.01                 | Do.                        |
| Do                          | 0.25                          | 0.01                 | Fair, some visible cracks. |
| Do                          | 0.5                           | 0.01                 | Good, no cracks.           |
| Do                          | 1.0                           | 0.01                 | Do.                        |
| Do                          | 7.0                           | 0.01                 | Do.                        |
| Do                          | 15.0                          | 0.01                 | Do.                        |
| Do                          | 25.0                          | 0.85                 | Do.                        |

<sup>1</sup> American Iron and Steel Substitute.

The data presented in the foregoing table show that the employment of sulfur in the welding flux during welding operations effectively inhibits loss of metal when the welding specimen is subjected to a boiling Straus solution. The data further show that the stressing of the tested specimen produces less detrimental effect in the metals welded in the presence of flux containing 0.25% to 25% by weight of elementary sulfur than the weld conducted in the absence of elementary sulfur in amounts up to 0.25% by weight.

It may be concluded from the results of the Straus test that elementary sulfur in the amounts stated in the welding flux effectively inhibits carbide formation and precipitation of carbides at the grain boundaries of the alloys and, therefore, substantially reduces susceptibility to intergranular corrosion.

The mechanism of the process is not fully understood; however, it is postulated that sulfur and sulfur compounds inhibit metallic carburization and metal carbide formation; thus,

chromium carbide is never formed in the process and, therefore, there are no chromium "lean" areas in the alloy after welding, this allows the alloy to retain its original corrosion resistant characteristics.

The welding fluxes to which the sulfur is added are the welding fluxes commonly used in welding stainless steels. Usually these welding fluxes are composed of some compound of the silicates, oxides, hydroxides, halides, carbonates, etc. of magnesium, calcium, sodium, potassium, lithium, and other alkali or alkaline earth metals along with small amounts of salts of titanium, manganese, columbium, vanadium, etc.

15 The welding fluxes mentioned above may have elementary sulfur in an amount in the range from 0.25% to 25% by weight incorporated therein and then applied either to the welding rod or to the region being welded. It is contemplated and 20 may be preferred that the welding flux containing elementary sulfur may be applied as a coating to welding rods in a weight ratio of welding flux coating on the welding rod in the range from 1:2 to 1:4 parts by weight.

25 The welding rods employed in the practice of the present invention may have a composition substantially the same as the stainless steel being welded. It may be preferred under some conditions, however, that the welding rods contain higher proportions of nickel and/or chromium than the alloy being welded. For example, when welding 18-8 steel it may be desirable to use 18-8 welding rods coated with a welding flux in accordance with the present invention or use 19-9 or 25-20 welding rods. A welding rod of 18-8 or 30 19-9 stainless steel having a coating of 1 part by weight of welding flux of the type illustrated to 2 parts by weight of welding rod gives quite satisfactory results in the present invention.

35 40 When employing a flame in the welding operation the gases may be acetylene or the liquefied petroleum gases, such as propane, butanes, butylenes, propylene, mixtures thereof, and the like.

45 While the oxy-acetylene torch may be used in the welding operation, the invention is equally applicable to electrical arc welding technique since most steels and alloys of the type mentioned above contain carbon which allows the formation of carbides in the welding operation. The invention is also applicable to welding using atomic hydrogen as a source of heat.

50 The nature and objects of the present invention having been fully described and illustrated, what I wish to claim as new and useful and to secure by Letters Patent is:

55 1. A method of welding a chrome-nickel stainless steel which includes the steps of applying a mixture of a conventional welding flux containing elementary sulfur in an amount in the range between 0.25% and 25% by weight, to two adjacent boundaries of bodies of said steel and welding said adjacent boundaries in the presence of said mixture.

60 65 2. A method in accordance with claim 1 in which the steel is welded by applying an electric arc to the adjacent boundaries of bodies of said steel.

70 75 3. A method in accordance with claim 1 in which the steel is welded by applying an oxy-acetylene flame to the adjacent boundaries of bodies of said steel.

4. A method in accordance with claim 1 in which the steel is welded by applying a hydrocarbon flame to the adjacent boundaries of bodies of said steel.

5. A method of welding a chrome nickel stain-  
less steel which includes the steps of forming a  
mixture of a conventional welding flux and ele-  
mentary sulfur, said mixture containing between  
0.25% and 25% by weight of elementary sulfur, 5  
applying said mixture to two adjacent boundaries  
of bodies of said steel, and welding said adjacent  
boundaries in the presence of said mixture.

6. A method in accordance with claim 5 in  
which the steel is welded by applying an oxy- 10  
acetylene flame to the adjacent boundaries of  
bodies of said steel.

PRENTISS S. VILES.

**References Cited in the file of this patent**

UNITED STATES PATENTS

| Number    | Name   | Date          |
|-----------|--------|---------------|
| 1,720,039 | Green  | July 9, 1929  |
| 2,141,929 | Moritz | Dec. 27, 1938 |

| Number    | Name          | Date           |
|-----------|---------------|----------------|
| 2,231,917 | Jones         | Feb. 18, 1941  |
| 2,329,986 | Goodford      | Sept. 21, 1943 |
| 2,468,371 | Landis et al. | Apr. 26, 1949  |
| 2,468,372 | Landis        | Apr. 26, 1949  |
| 2,473,601 | Lobosco       | June 21, 1949  |

FOREIGN PATENTS

| Number           | Country       | Date          |
|------------------|---------------|---------------|
| 1,403<br>of 1909 | Great Britain | Jan. 20, 1910 |
| 467,450          | Great Britain | June 17, 1937 |
| 541,446          | Great Britain | Nov. 27, 1941 |

OTHER REFERENCES

15 Alloys of Iron and Chromium, by Kinsel and  
Franks. Vol. 2, p. 181 (103, Weld). Pub. by  
McGraw-Hill Book Co., New York, N. Y. (Copy  
in Div. 3.)